

# UNITED STATES PATENT OFFICE.

CHARLES J. POWNALL, OF ADDISON ROAD, KENSINGTON, ENGLAND.

## IMPROVEMENT IN PROCESSES FOR PREPARING VEGETABLE FIBER.

Specification forming part of Letters Patent No. 9,650, dated April 5, 1852.

*To all whom it may concern:*

Be it known that I, CHARLES JAMES POWNALL, of Addison Road, in the county of Middlesex, England, gentleman, have invented or discovered new and useful Improvements in the Treatment and Preparation of Flax and other Similar Fibrous Vegetable Substances; and I, the said CHARLES JAMES POWNALL, do hereby declare that the nature of my invention and the manner in which the same is to be performed are particularly described and ascertained in and by this present specification thereof, as follows—that is to say:

My said invention consists of a mode or modes of preparing or treating flax and other similar fibrous vegetable substances for the purpose of depriving them more effectually of their resinous and gummy matters, and, when required, for the purpose of resolving them, or the ordinary filaments of those substances, into their ultimate fibers. For this purpose I adopt a mode or modes of treating those substances, not only for the purpose of more effectually removing such resinous or gummy matters, as aforesaid, but also for the purpose of separating the more minute fibers of which they are composed from each other without the aid of any injurious chemical agents, and without cutting, tearing, or in any way injuring those minute fibers, and thus obtaining a fibrous material of great fineness.

When I apply my process to flax I take the retted straw and subject it to the process which I am about to describe. I prefer, however, that the flax upon which I operate should be scutched, so as to remove the boon or wood from it before it is retted, for the purpose not only of getting rid of the boon or wood more effectually, but also diminishing the bulk of the material to be operated upon and causing the mechanical action hereinafter mentioned to be more effectually applied to the filaments of the flax to be operated upon.

The flax may be retted or fermented according to any of the known methods; but I must observe that the more perfectly the retting process is performed the more easily will the minute fibers of the plant be separated from each other; and in performing the retting process upon the straw of flax intended to be submitted to my process I deem it desirable to conduct it in such a manner as to prevent the acetous fermentation of that process passing

into such a stage as will cause it to injure or discolor the fibrous matters of the vegetable, and for this purpose, from time to time, during the progress of the retting or fermentation, as the resinous, glutinous, and other matters separated from the vegetable rise to the top of the tank, or vessel, or pit in the state of scum, I remove such scum, and also change, or partially change, the water for the purpose of preventing or checking any tendency of the flax or the matters extracted from it to pass into the putrid or destructive fermentation.

When the retting process has been effectually performed upon the straw of flax the lint or ordinary filaments of the flax may be easily separated from the boon or wood with which it is mixed by any of the ordinary means used for that purpose. Instead of drying the retted material immediately after it has been retted, as is now usually done, I adopt the following mode of treatment for more effectually removing the residue of its resinous or gummy matters: For this purpose I place the retted flax in a suitable machine or vessel, through which I cause a stream of water to flow, and in which the flax is subjected to a powerful mechanical action, and is repeatedly beaten, pressed, or squeezed until all the resinous or gummy matters are as much as possible removed from it.

Instead of losing only from fifteen to twenty per cent. of the weight, as when treated in the ordinary way, the flax will be deprived of the whole, or nearly the whole, of its resinous or gummy matters, amounting to about forty per cent., by the retting and the process just mentioned. The machine which I prefer to use for this purpose is made upon the well-known principle of the tuck or fulling mill, and taking care that there shall be a sufficient supply of water running through the flax to wash away the resinous or gummy matters as they are detached from the flax by the operation of the machinery. If the flax has not been scutched before it was retted, I now proceed to dry it in a chamber heated with steam-pipes or other convenient means, for the purpose of enabling me to get rid of the boon or wood; and when thoroughly dry I pass the flax through heavy rollers, as at present, so as to break or crush the whole of the wood or boon and detach it from the filaments of the flax, and then I scutch it by any convenient machinery, so as to remove the woody parts and obtain the fila-

ments of the flax in a separate state. If the flax has been scutched before retting, it may, if desired, be bleached by any ordinary means before it is dried. I then cause the scutched or dried material to be passed through a machine usually called a "wool willow," or some similar machine, for the purpose of "opening out" the material and dividing the lumps or masses in such a manner as to make it more fit for combing or carding or other process, according to the use to which it may be intended to be applied.

If I desire to separate the filaments of the flax into their ultimate or finer fibers I then proceed to card it; and the resinous or gummy matters having been removed by the process already described, the filaments of the flax will separate into the ultimate or finer fibers of which they are composed, and the fibrous matter thus obtained may be spun upon any suitable machinery. The fibers into which filaments of flax may be thus separated are very fine, and I have ascertained that the fibers contained in a plant are nearly uniform in length, such lengths varying from about three-fourths of an inch to about two and a half inches, according to the growth of the flax-plant; that they have tapering ends, and are in every way fitted for being spun into threads. By pursuing this mode of obtaining the finer or ultimate fibers I avoid cutting or tearing them.

and am thus enabled to obtain them in a better state for spinning into threads which may be used in the manufacture of many textile fabrics, and for other purposes.

The mode of treating hemp and other fibrous vegetable matters is precisely similar to that which I have described with reference to flax, and the vegetable matters operated upon in this way may, in addition, be bleached by any ordinary process applicable for that purpose.

Having now described the nature of my said invention and the manner of performing the same, I hereby declare that I claim as of my invention—

The mode of subjecting fibrous vegetable substances to repeated mechanical pressure and the action of a stream of water for the purpose of depriving them of resinous or gummy matters, and also resolving them into their ultimate or finer fibers, in manner hereinbefore described.

In witness whereof I, the said CHARLES JAMES POWNALL, have hereunto set my hand this 5th day of August, 1852.

CHAS. J. POWNALL.

Witnesses:

R. A. WROOMAN,  
*Patent Agent, 106 Fleet St., London.*  
JNO. COOK,  
*Curzon Street, London.*